

# UNITED STATES PATENT OFFICE.

DAVID L. MCKENZIE, OF WINNIPEG, MANITOBA, CANADA.

## LUBRICATING COMPOUND.

SPECIFICATION forming part of Letters Patent No. 351,195, dated October 19, 1886.

Application filed June 10, 1886. Serial No. 204,720. (No specimens.)

*To all whom it may concern:*

Be it known that I, DAVID L. MCKENZIE, of Winnipeg, Manitoba, Canada, have invented a new and useful Improvement in Lubricating Compounds, of which the following is a specification.

My invention is in the nature of an improved lubricating compound for car-axle boxes, journal-boxes, and all sliding bearings, designed to reduce friction to a minimum, and to preserve for a long time its lubricating qualities without decomposition or deterioration.

In preparing my compound I take the following ingredients and proportions: Animal fat, five per cent., by weight; mineral-oil refuse, seventy-five per cent., by weight; slaked lime, fifteen per cent., by weight; manganese, (black oxide,) five per cent., by weight. These I mix thoroughly together by heating to boil-

ing, and the compound is then ready to be put up for use, which compound is, when cool, about the consistency of paste or of a semi-fluid character.

It is not necessary that the exact proportions named should be adhered to, as a little more or less of any of the ingredients will not involve any substantial departure from my invention.

Having thus described my invention, what I claim as new is—

The lubricating compound herein described, consisting of animal fat, mineral-oil refuse, slaked lime, and manganese, in or about the proportions named.

DAVID L. MCKENZIE.

Witnesses:

EDWD. W. BYRN,  
SOLON C. KEMON.